

June 24, 1930.

C. L. MCKESSON

1,768,366

PROCESS FOR RETAINING WATER IN CONCRETE FOR THE HYDRATION OF CEMENT

Filed July 2, 1928



FIG. 1.

FIG. 2.



INVENTOR.

*Claude L. McKesson*

## UNITED STATES PATENT OFFICE

CLAUDE L. MCKESSON, OF SACRAMENTO, CALIFORNIA, ASSIGNOR TO AMERICAN BITUMULS COMPANY, OF SAN FRANCISCO, CALIFORNIA, A CORPORATION OF DELAWARE

## PROCESSES FOR RETAINING WATER IN CONCRETE FOR THE HYDRATION OF CEMENT

Application filed July 2, 1928. Serial No. 289,844.

The object of my invention is to provide simple, efficient and inexpensive means for retaining in concrete sufficient of the mixing water during the period following the placing thereof to insure the proper hydration of the cement and the development of the required tensile and compressive strengths. This beneficial result is accomplished without permanently discoloring the concrete. 5 Incidental to the conservation of water during the curing period and without additional expense it also provides means by which markings may be produced on the surface concrete pavement and bridges for 10 traffic direction or other purposes.

The process and means by which these and other beneficial results are obtained are described herein and are shown in the accompanying drawings in which

20 Fig. 1 shows one method of placing a covering of paper, felt, fabric or similar material on a freshly finished concrete pavement.

Fig. 2 shows a fragmental cross section 25 of pavement with completed protective covering in place. This section is taken on the dotted line A. A. in Fig. 1.

Throughout the views like characters refer to the like elements.

30 In the drawings 1 indicates a body of freshly placed concrete. 2 refers to a layer of granular mineral paper, felt, or other covering material which is placed directly upon the surface of the concrete such materials being generally absorbent or of water-

35 pervious nature. 3 indicates a second layer of paper, felt, fibrous or fabric covering material which is sometimes superimposed upon material 2. 4 is a surface coating of 40 waterproofing material such as tar, asphalt, or petroleum residuum preparation, which is spread over the cover material. 5 is a space between the edges of parallel strips of the coverings 2 and 3 which permits the

45 waterproofing material spread over the surface to come into contact with the surface of the concrete between the parallel strips to which it adheres and remains after the removal of the coated cover materials 2 and 50 3, forming thereby a traffic guide line upon

the light colored natural surface of the concrete.

The method of application of the treatment is briefly described as follows:

The material 2 is first spread upon the 55 freshly placed concrete. The cover material 2 may consist of sand or similar granular mineral matter. In such case only the one layer is needed. When paper, felt, or other pliable material is used it is sometimes 60 desirable to place it in two successive layers on the concrete. This method is illustrated in Fig. 1 and the first layer is designated as 2, the second layer as 3. The placing of pliable material is conveniently accomplished by having the cover material in rolls, 65 as shown in Fig. 1, so placed that successive and interlapping layers may be placed following the finishing of the concrete. The presence of this covering has the immediate 70 effect of protecting the surface of concrete from wind, sun, or injury from showers. The next stage which usually follows within a period of from a few minutes to several 75 hours consists of the application on the said covering already placed of a thin layer or film of waterproof material such as asphalt, petroleum residue, tar, varnish, or lacquer. Asphalts, cut back or emulsified asphalt, are generally most economical and preferably 80 the latter is used because, already containing water it has a natural affinity for the covering which is, by the time of its application, damp with moisture from the wet concrete.

85 Under unusual conditions the placing of the bituminous layer 5 may be deferred for a period during which the coverings 2 and 3 are kept wet by sprinkling with water. In this way additional water may be supplied to aid in hydration.

If the cover is allowed to remain a considerable period before waterproofing without sprinkling with water it will tend, by evaporation, to reduce the water content in 90 the surface of the concrete, a desirable accomplishment with very wet concrete.

95 After the hydration of cement in the concrete has progressed to the desired point the coverings 2 and 3 are removed from the 100

pavement taking with them the waterproof coating 4. This leaves the concrete clean and free from discoloration except where, as stated, an opening 5 has been left between 5 parallel strips of cover material to permit the waterproofing material to reach the concrete to which it adheres and produces the guide line, as stated.

The exact thickness or kind of material 10 used in coverings 2 and 3 is not essential to this invention. Usually very thin inexpensive paper meets the requirements. The number of layers may be varied to meet the conditions prevailing on the work. A single 15 layer 2 coated with a waterproof coating 4 is somewhat more difficult to remove; otherwise, it satisfactorily accomplishes the purpose.

Granular material such as sand or earthy 20 matter ordinarily available adjacent to highway construction also affords an economical and satisfactory cover material. In such case the cover material may be spread on the wet concrete to any desired thickness and covered with bituminous emulsion or other 25 liquid asphaltic material with or without prior application of additional water. In due time after the curing of the concrete has been effected the cover material with its asphaltic coating may be disintegrated and 30 swept to the sides of the roadway where it may be compacted to provide shoulders wherein the binding qualities of the disintegrated asphalt may be utilized.

35 Having thus described my invention what I claim as new and desire to secure by Letters Patent is:

1. The process of retaining water in concrete for hydration of cement by placing 40 water-pervious cover material on the surface of the concrete and by applying to said cover material a treatment of non-absorptive material.

2. The process of retaining water in concrete for hydration of cement by covering 45 the concrete with material which will not permanently adhere to the concrete and by treating said material with a coating of material of a waterproofing nature adapted to 50 resist the passage of water or water vapor from the concrete.

3. The process of retaining water in concrete for hydration of cement by placing a removable protective covering on the concrete 55 and by coating said protective covering with waterproofing material adapted to retard passage of moisture through the said protective coating.

4. The process of retaining water in concrete for hydration of cement by covering the concrete with a porous material and by applying to said porous material a surface treatment of waterproofing adapted to prevent evaporation through said porous material of water contained in the concrete.

5. The process of retaining water in concrete for hydration of cement by placing thereon successive layers of pliable cover material adapted to come into close contact with the surface of said concrete and by distributing on the uppermost of said cover material a coating of liquefied bituminous material. 70

6. The process of retaining water in concrete for hydration of cement by placing 75 thereon cover material, said cover material being so placed as to leave the bare surface of the concrete between the edges thereof at predetermined intervals for the purpose of forming traffic markings and a liquid waterproofing treatment applied to the surface of the said cover material and to the exposed concrete between the edges of the cover material, adapted to retard the escape of moisture from the concrete. 80

85 7. The process of retaining water in concrete for hydration of cement by covering said concrete with removable cover material and by coating the said cover material with liquefied asphaltic material of a type which will produce a water resistant film on the surface of said cover material all substantially as described and for the uses and purposes set forth. 90

95 8. A process of curing hydraulic cement concrete which comprises covering the concrete while still wet with absorbent material, applying water to said absorbent material, applying waterproofing material to the surface of said absorbent material to retard the loss of water during the curing period and removing said absorbent material and waterproofing material from the cured concrete. 100

105 9. A process of curing hydraulic cement concrete which includes applying a layer of water-pervious material while the concrete is still wet, applying bituminous emulsion to substantially seal the surface of the water-pervious material during the curing period and removing the water-pervious material and sealing material from the cured concrete. 110

115 CLAUDE L. MCKESSON.

115

120

125

130